

94-22

SEARCHED FOR MISSING COPY

SEARCHED

106/83

X 13P/128  
X 106/83

# UNITED STATES PATENT OFFICE.

A. VAN CAMP, OF WASHINGTON, DISTRICT OF COLUMBIA, AND M. M. HODGMAN, OF ST. LOUIS, MISSOURI.

## IMPROVEMENT IN CONCRETE FOR PAVEMENTS AND FOR OTHER PURPOSES.

Specification forming part of Letters Patent No. 96,850, dated November 16, 1869.

518

To all whom it may concern:

Be it known that we, A. VAN CAMP, of Washington city and District of Columbia, and M. M. HODGMAN, of St. Louis, in the county of St. Louis and State of Missouri, have invented a certain new and useful Improvement in Concrete Composition for Pavements, Roofs, Pipes, Drains, &c.; and we do hereby declare that the following is a full, clear, and exact description of the same.

The nature of our invention consists in so mixing asphaltum, or the residuum of pitch or coal-tar, decomposed silex, and sand together that a composition is formed, the concretion of which is of such character as to render it most admirably adapted for the purposes of paving, roofing, flooring, water and drain pipes, &c.

A pavement laid of this composition, practical experience has fully proven to be entirely free of the whole series of objections which justly exists against those compositions now commonly styled "concrete pavements."

In a vast majority of these compositions, the spontaneous adhesion, as it were, of the different ingredients, which is positively necessary to produce concretion, does not take place. The result is, that disintegration of the ingredients soon occurs, and, as a consequence, when the pavement is subjected to the action of severe frost, or the direct rays of the sun, it soon begins either to so shrink or swell as to be perfectly worthless. Nor is this at all remarkable, when the fact is taken into consideration that the chief ingredient—at least, the ingredient which possesses the cementing property in so many cases—is ordinary coal-tar, or like evaporating material. The asphaltum or residuum of coal-tar which we use does not evaporate, and, therefore, its adhesive qualities are never wasted, and, when mixed with sand and decomposed silex, as hereinafter stated, will produce a pavement or walk, roofing or pipe, perfectly impervious to and entirely unaffected by moisture. It will alike resist the action of intense heat or cold, its materials so coalescing, when once mixed and laid, that it becomes a positive solid mass, the decomposed silex causing each and every interstice, no matter how minute the same may be, to be filled, and one that it

is utterly impossible for the frost to enter, much less embed itself in. The result is, that the pavement is firm and durable, presenting a level and uniform surface during all seasons; and, while it will resist, in a remarkable degree, all attrition, at the same time it is sufficiently elastic to prevent the animal slipping; and, as it wears, the mass being of the same consistency all through, a like surface is always presented.

To enable others skilled in the art to make and use our invention, we will now proceed to describe its method of construction.

We take, of coarse and fine sharp sand, five pounds each, and of decomposed silex, one pound. These we place in an iron pan or other suitable vessel, and heat to, say, about 150° or 160°. We then take of the asphaltum or the residuum three pounds, and melt the same.

These proportions, as well as the degree of heat, of course, may be varied, each being increased or diminished at pleasure, or as may be deemed desirable.

So soon as the asphaltum or the residuum is reduced to a state sufficiently plastic, the mixing should take place. The asphaltum is then poured gradually in upon the sand and decomposed silex, the latter being subjected to heat, and the mass undergoing thorough agitation during the entire process. After the mass has been duly heated and properly mixed, it is to be instantly laid, as we always use the composition while it is yet in a warm, plastic state.

The pavement is laid by hot tamps and hot rollers, similar to the manner described in our patent before referred to.

As to the quantity of the materials used in the composition, practical experience has fully attested the fact that the formula heretofore given, as a general rule, gives the proper proportions; but, as asphaltum and residuum vary in quality, some containing much more oil than others, the quantity of asphaltum to be added to the sand and decomposed silex will require to be greater or less, as the case may be, it depending entirely on the quality of the article used.

The composition herein described is applicable and most admirably adapted for water and drain pipes.

• 6,650

The pipes are formed in hot molds, of suitable dimensions, the necessary pressure being applied from within.

Having thus fully described our invention, what we claim therein as new, and desire to secure by Letters Patent of the United States, is—

1. A concrete composition for paving, roofing, flooring, &c., when the same is composed of asphaltum or the residuum of pitch or coal-tar, sand, and decomposed silex, substantially as described.

2. Laying the composition, herein described,

for a pavement or walk by means of hot tamps and hot rollers, substantially as described.

3. A water or drain pipe, when the same is composed of the composition herein described.

In testimony whereof we have signed our names to this specification in the presence of two subscribing witnesses.

A. VAN CAMP.  
M. M. HODGMAN.

Witnesses:

EDWIN JAMES,  
EDM. F. BROWN.

1861/23

silica